

# United States Patent Office

3,316,085

Patented Apr. 25, 1967

1

3,316,085

**MARTENSITIC STAINLESS STEEL**  
 Willard E. Grundman and Mary E. Potter, Thornton Township, Cook County, Ill., assignors to United States Steel Corporation, a corporation of Delaware  
 No Drawing. Filed May 21, 1964, Ser. No. 369,286  
 2 Claims. (Cl. 75—128)

This application relates to martensitic stainless steels suitable for pressure vessel applications and more par-

2

structure and then tempered at about 1100 to 1150° F. Tempering at such temperature is desired to produce optimum resistance to stress corrosion cracking and is used with the steel of this invention to obtain the required minimum tensile and impact properties. Tempering at temperatures of the order of 1200° F. tends to reduce the tensile strength below the minimum required value.

To illustrate the properties obtained by following the teachings of our invention, steels of the following composition were made and tested as hereinafter described:

TABLE I

| Heat No.  | Chemical Composition, Weight Percent |      |       |       |      |       |      |      |      |      |
|-----------|--------------------------------------|------|-------|-------|------|-------|------|------|------|------|
|           | C                                    | Mn   | P     | S     | Si   | Cr    | Ni   | Mo   | V    | W    |
| 1         | 0.11                                 | 0.47 | 0.007 | 0.009 | 0.23 | 12.60 | 2.01 | 1.30 | 0.25 | —    |
| 2         | 0.14                                 | 0.29 | 0.012 | 0.006 | 0.55 | 12.88 | 1.99 | 1.56 | 0.27 | —    |
| 3         | 0.15                                 | 0.29 | 0.015 | 0.007 | 0.61 | 12.50 | 2.02 | 1.54 | 0.36 | —    |
| 4         | 0.19                                 | 0.50 | 0.006 | 0.015 | 0.46 | 12.15 | 2.15 | 1.44 | 0.35 | —    |
| 5         | 0.22                                 | 0.48 | 0.015 | 0.007 | 0.56 | 12.52 | 1.87 | 1.44 | 0.55 | —    |
| 6         | 0.11                                 | 0.11 | 0.007 | 0.012 | 0.22 | 11.84 | 1.91 | 1.52 | 0.17 | —    |
| 7         | 0.11                                 | 0.48 | 0.005 | 0.016 | 0.52 | 12.53 | 2.02 | 1.52 | 0.57 | —    |
| 8         | 0.12                                 | 0.11 | 0.007 | 0.011 | 0.25 | 11.84 | 1.91 | 1.48 | 0.18 | —    |
| 9         | 0.14                                 | 0.17 | 0.005 | 0.009 | 0.35 | 11.99 | 2.00 | 1.48 | 0.21 | —    |
| Type: 422 | 0.20                                 | 0.65 | —     | —     | 0.50 | 12.00 | 1.00 | 0.75 | 0.30 | 1.00 |

ticularly to martensitic stainless steels having high tensile strength combined with good impact properties after tempering.

For many pressure vessel applications, steels having a minimum room temperature tensile strength of 160,000 p.s.i. combined with a Charpy V-notch impact strength of 15 foot-pounds at -40° F. are required in the tempered condition in heavy plates up to 4 inches in thickness. We have discovered that such combination of properties can be obtained in martensitic stainless steel containing prescribed amounts of carbon, nickel, molybdenum and vanadium. Thus the desirable combination of properties may be obtained in steel containing the following elements within the ranges listed by weight percent:

|            | Wt. percent |
|------------|-------------|
| Carbon     | 10.25       |
| Manganese  | 10.60       |
| Silicon    | 20.80       |
| Chromium   | 11.00-14.00 |
| Nickel     | 1.5-2.5     |
| Molybdenum | 1.0-2.0     |
| Vanadium   | .25-.55     |

wherein the vanadium content is in excess of .35% with carbon contents in excess of .15% with the balance iron and other elements in amounts which do not adversely affect the properties.

Preferably the steel should be within the following compositional ranges by weight percent:

|            | Wt. percent |
|------------|-------------|
| Carbon     | .13-.15     |
| Manganese  | .25-.60     |
| Silicon    | .20-.50     |
| Chromium   | 12.00-12.75 |
| Nickel     | 1.75-2.25   |
| Molybdenum | 1.40-1.60   |
| Vanadium   | .25-.35     |

with the balance iron and residual impurities.

The steel should be austenitized at about 1850° F. or above for at least sufficient time to cause the steel to be substantially completely austenitic. Thereafter it is cooled at a sufficiently rapid rate to transform it to a martensitic

These heats were forged at 2100° F. to 1-inch diameter round bars and 1/2-inch square bars and tested as indicated in the following Table II:

TABLE II

| Heat No.  | Room Temperature Tensile Properties |                           |                            | Impact Strength, Charpy V-notch, ft./lb. |            |
|-----------|-------------------------------------|---------------------------|----------------------------|------------------------------------------|------------|
|           | Tensile Strength, p.s.i.            | Elongation in 2", percent | Reduction of Area, percent | -40° F.                                  | Room Temp. |
| 1         | 161,000                             | 15.0                      | 57.7                       | 20                                       | 49         |
| 2         | 169,385                             | 16.0                      | 57.8                       | 20                                       | 36         |
| 3         | 175,100                             | 15.5                      | 55.7                       | 18                                       | 36         |
| 4         | 167,125                             | 15.0                      | 51.6                       | 20                                       | 37         |
| 5         | 165,425                             | —                         | —                          | 17                                       | —          |
| 6         | 132,350                             | 18.0                      | 57.7                       | —                                        | —          |
| 7         | 154,325                             | 18.0                      | 62.8                       | —                                        | —          |
| 8         | 140,300                             | 17.0                      | 53.2                       | —                                        | —          |
| 9         | 158,350                             | 14.0                      | 47.8                       | —                                        | —          |
| Type: 422 | 150,000                             | 17.0                      | 53.0                       | —                                        | —          |

Heat Treatment: 30 minutes at 1800° F., air cool plus tempering for 4 hours at 1100° F., air cool.

As indicated by the foregoing Table II, steels of this invention develop the required tensile and impact properties after austenitizing at 1800° F. and air cooling to room temperature followed by tempering for 4 hours at 1100° F. and air cooling to room temperature. As further indicated by these results, the carbon and vanadium contents are critical to the desired results. With carbon in excess of .15%, the vanadium content must exceed .35%. The desired results can be obtained with carbon and vanadium increased above the preferred range but with no advantage in results and of course with the added expense of the increased vanadium.

The published composition of Type 422 is included in Table I and its properties in Table II for comparative purposes. As shown, the required properties are not obtained with the conventional AISI Type 422 which exhibits the highest strength of the standard 12% chromium steels after austenitizing, air cooling and tempering in the range of 1100 to 1150° F.

While we have shown and described several specific embodiments of our invention, it will be understood that these embodiments are merely for the purpose of illustra-

tion and description and that various other forms may be devised with the scope of our invention, as defined in the appended claims.

We claim:

1. Martensitic stainless steel characterized by a room temperature tensile strength in excess of 160,000 p.s.i. and a Charpy V-notch impact strength in excess of 15 foot-pounds at minus 40° F. after austenitizing and tempering, said steel consisting essentially of

|            | Wt. percent | 10 |
|------------|-------------|----|
| Carbon     | .10-.25     |    |
| Manganese  | .10-.60     |    |
| Silicon    | .20-.80     |    |
| Chromium   | 11.00-14.00 |    |
| Nickel     | 1.5-2.5     | 15 |
| Molybdenum | 1.0-2.0     |    |
| Vanadium   | .25-.55     |    |

wherein with the carbon content in excess of .15% the vanadium content is in excess of .35% with the balance 20 iron and residual impurities.

2. Martensitic stainless steel characterized by a room temperature tensile strength in excess of 160,000 p.s.i. and a Charpy V-notch impact strength in excess of 15 foot-

pounds at minus 40° F. after austenitizing and tempering, said steel consisting essentially of

|            | Wt. percent |
|------------|-------------|
| Carbon     | .13-.15     |
| Manganese  | .25-.60     |
| Silicon    | .25-.50     |
| Chromium   | 12.00-12.75 |
| Nickel     | 1.75-2.25   |
| Molybdenum | 1.40-1.60   |
| Vanadium   | .25-.35     |

with the balance iron and residual impurities.

#### References Cited by the Examiner

##### UNITED STATES PATENTS

|           |         |          |          |
|-----------|---------|----------|----------|
| 1,630,448 | 5/1927  | Oertel   | 75-128   |
| 1,787,403 | 12/1930 | Strauss  | 75-128 X |
| 2,227,891 | 1/1941  | Rose     | 75-128   |
| 2,306,421 | 12/1942 | Arness   | 75-128 X |
| 2,695,229 | 11/1954 | Sheridan | 75-128   |

HYLAND BIZOT, Primary Examiner.

DAVID L. RECK, Examiner.

P. WEINSTEIN, Assistant Examiner.

UNITED STATES PATENT OFFICE  
CERTIFICATE OF CORRECTION

Patent No. 3,316,085

April 25, 1967

Willard E. Grundman et al.

It is hereby certified that error appears in the above numbered patent requiring correction and that the said Letters Patent should read as corrected below.

Column 2, line 8, for "illustrated" read -- illustrate --;  
line 41, Table II, sixth column, line 1 thereof, for "49" read  
-- 46 --; column 3, line 2, for "with" read -- within --;  
column 4, line 6, for ".25" read -- .20 --.

Signed and sealed this 21st day of November 1967.

(SEAL)

Attest:

Edward M. Fletcher, Jr.

Attesting Officer

EDWARD J. BRENNER

Commissioner of Patents